

## UNITED STATES PATENT OFFICE

2,405,581

## FLOTATION OF SULPHIDE ORES

Cornelius H. Keller, San Francisco, Calif., assignor to The Dow Chemical Company, Midland, Mich., a corporation of Michigan

No Drawing. Application October 17, 1944,  
Serial No. 559,117

11 Claims. (Cl. 209—166)

1

This invention relates to the concentration of ores, minerals and the like by flotation, and has for its broad object the provision of certain improvements in the process.

In the froth flotation of ores, an ore pulp is first prepared by wet grinding to a suitable size with or without a suitable pH modifier. A suitable frothing agent and a flotation agent are then added. Upon agitating and aerating the mixture, the metalliferous values in the ore collect as a froth which can be readily overflowed or skimmed off and the metal values therein recovered.

Flotation agents, as a broad class, are well known. Generally within the broad class sub-classification is possible into several groups, each of which will differ from another in its flotation effect. The present invention is concerned with a group of agents which are not only good collectors, but are also highly selective in their action, enabling sulphide copper minerals, sulphide zinc minerals and others to be floated selectively from sulphide iron minerals. The new agents are obtained as the reaction product of a carbocyclic acid halide, a monohydric aliphatic alcohol and an alkali thiocyanate, the chemical constitution of which is not fully known. These possess numerous advantages. For example, they are soluble to a useful extent in various organic solvents, such as amyl alcohol and cresylic acid, thereby enabling the agent to be fed as a liquid. Further, these agents can be incorporated and utilized with other agents such as xanthates. When treated with an alkali hydroxide, these agents are converted into water soluble salts which can be fed as water solutions.

The materials of the present invention are conveniently prepared by the interaction of any carbocyclic acid halide such as benzoyl chloride, benzoyl bromide, furoyl chloride, furoyl bromide, or other carbocyclic acid halide upon an alcoholic solution or suspension of an alkali thiocyanate such as potassium thiocyanate, ammonium thiocyanate, sodium thiocyanate. Any aliphatic monohydric alcohol can be used and I have successfully employed ethyl, isopropyl, secondary butyl, N-amyl, N-butyl, octyl and a mixture of amyl alcohols (sold under the trade-name "Pentasol") and diethylcarbinol.

A typical example of the preparation of these materials follows:  $\frac{1}{2}$  mol. weight of a suitable alkali thiocyanate was triturated in a mortar with  $\frac{1}{2}$  mol. weight of the selected alcohol. When these were ground and mixed,  $\frac{1}{2}$  mol.

2

weight of the organic acid halide was added very slowly under continued trituration. The mass, at first milky, assumed a canary yellow color which gradually changed to a deep orange. This reaction was accompanied by a rise in temperature. This ceased when the orange color appeared, showing that the reaction was completed. The product consists of organic sulphur compounds of undetermined composition.

10 To illustrate some of the advantages to be gained by the use of the crude reaction product collecting agents as compared to the principal and best known collecting agent, namely xanthate, the following examples are set forth:

15 As a general procedure the sample of ore was ground wet in a ball mill with a suitable pH modifier. When sufficiently ground, the pulp was transferred to either a Fagergren or a Denver Sub A flotation machine and the flotation reagent and frother were added. The pulp was then subjected to agitation and aeration and the froth concentrate was removed.

The designation "R. P." is employed in the following tables to indicate the reaction product.

20 To illustrate the present invention, charges of copper ore from Utah were prepared and treated, comparison being made between the various chemical flotation reagents contemplated by this invention and potassium ethyl xanthate as collector:

Tabulation #1—Copper ore from Utah

| 35 | Flotation reagent used                                        | Lbs./ton | Concen-<br>trate<br>per cent<br>copper | Tailings<br>per cent<br>copper | Copper<br>recovery<br>per cent<br>in con-<br>centrate |
|----|---------------------------------------------------------------|----------|----------------------------------------|--------------------------------|-------------------------------------------------------|
| 40 | K ethyl xanthate                                              | 0.1      | 12.2                                   | 0.1                            | 88.8                                                  |
|    | NaCNS ethylalcohol                                            |          |                                        |                                |                                                       |
|    | benzoylchloride R. P.                                         | 0.05     | 19.12                                  | 0.11                           | 90.0                                                  |
|    | NaCNS-N, amylalcohol                                          |          |                                        |                                |                                                       |
|    | benzoylchloride R. P.                                         | 0.1      | 14.08                                  | 0.09                           | 92.2                                                  |
|    | NaCNS-N, butylalcohol                                         |          |                                        |                                |                                                       |
|    | benzoylchloride R. P.                                         | 0.1      | 14.8                                   | 0.092                          | 91.3                                                  |
|    | NaCNS-N, amylalcohol                                          |          |                                        |                                |                                                       |
|    | furoylchloride R. P.                                          | 0.15     | 13.04                                  | 0.1                            | 90.3                                                  |
|    | NaCNS-N, butylalcohol                                         |          |                                        |                                |                                                       |
|    | furoylchloride R. P.                                          | 0.15     | 18.96                                  | 0.13                           | 87.6                                                  |
|    | NH <sub>4</sub> CNS-N, butylalco-<br>hol furoylchloride R. P. |          |                                        |                                |                                                       |
|    |                                                               | 0.15     | 8.28                                   | 0.095                          | 91.5                                                  |
|    | KCNS-octylalcohol ben-<br>zoylbromide R. P.                   | 0.1      | 10.12                                  | 0.062                          | 90.0                                                  |

LEGEND.—R. P. stands for Reaction Product.

<sup>1</sup> Emulsol used as a frother only with this reagent; cresylic acid being used in all other tests.

55 Comparing the results secured, it is to be

noted that the copper recovery is generally increased when the reaction product is employed instead of potassium ethyl xanthate.

To compare the value of the reaction product collecting agent with xanthates, a sulphide cop-

Illustrating the greater selectivity of water soluble alkali metal salts of the reaction products over xanthates, a sulphide copper from Utah was prepared for flotation and tested with the following results:

Tabulation #4.—Copper ore from Utah

| Flotation reagent used <sup>1</sup> | Lbs./ton | Concentrate     |               | Tails per cent copper | Copper recovery per cent in concentrate | Iron recovery per cent in concentrate |
|-------------------------------------|----------|-----------------|---------------|-----------------------|-----------------------------------------|---------------------------------------|
|                                     |          | Per cent copper | Per cent iron |                       |                                         |                                       |
| Potassium iso-propyl R. P.          | 0.02     | 22.4            | 13.7          | 0.12                  | 89.1                                    | 21.2                                  |
| Potassium secondary butyl R. P.     | 0.02     | 25.0            | 15.0          | 0.12                  | 89.5                                    | 21.4                                  |
| Potassium pentasol R. P.            | 0.02     | 25.2            | 15.1          | 0.13                  | 88.1                                    | 21.6                                  |
| Potassium diethylcarbinol R. P.     | 0.02     | 24.2            | 14.6          | 0.12                  | 89.6                                    | 21.3                                  |
| Pentasol xanthate                   | 0.02     | 16.8            | 21.1          | 0.12                  | 89.9                                    | 43.8                                  |
| Ethyx xanthate                      | 0.02     | 15.8            | 19.9          | 0.11                  | 90.2                                    | 46.4                                  |

<sup>1</sup> Cresylic acid used as a frother.

per ore from Arizona was used. The results are shown in the following table:

The selectivity with respect to iron is quite pronounced on this ore.

Tabulation #2.—Copper ore from Arizona

| Flotation reagent used <sup>1</sup> | Lbs./ton | Concentrate     |               | Tails per cent copper | Copper recovery per cent in concentrate | Iron recovery per cent in concentrate |
|-------------------------------------|----------|-----------------|---------------|-----------------------|-----------------------------------------|---------------------------------------|
|                                     |          | Per cent copper | Per cent iron |                       |                                         |                                       |
| R. P. isopropyl                     | 0.035    | 13.6            | 24.9          | 0.145                 | 86.26                                   | 51.4                                  |
| R. P. pentasol                      | 0.035    | 13.6            | 24.5          | 0.135                 | 86.81                                   | 51.62                                 |
| R. P. diethylcarbinol               | 0.035    | 13.6            | 23.8          | 0.135                 | 86.71                                   | 50.68                                 |
| K. ethyl xanthate                   | 0.05     | 12.32           | 30.4          | 0.17                  | 83.24                                   | 65.44                                 |
| K. amyl xanthate                    | 0.05     | 13.68           | 30.2          | 0.19                  | 81.13                                   | 56.27                                 |

R. P. flotation reagents were prepared from alcohol, benzoylchloride and NaCNS. Only the alcohol is indicated in tabulation.

<sup>1</sup> Fuel oil mix employed as a frother in each case.

The reaction product enables several per cent more copper to be recovered than does either the purified ester or even a larger quantity of either potassium ethyl xanthate or potassium amyl xanthate.

To demonstrate the collecting effectiveness and selectiveness of the reaction products dissolved in cresylic acid or amylalcohol as compared to xanthate, a sulphide copper ore from Arizona was prepared for flotation and treated, with the following results:

To illustrate the compatibility of the reaction products with xanthates and the greater selectivity obtained by the addition of the reaction products of this invention to xanthates, different percentages of the reaction products were added to xanthate in various stages of its preparation.

Also, a water soluble alkali salt of the reaction product was mixed with xanthate in different

Tabulation #3.—Copper ore from Arizona

| Flotation reagent used <sup>1</sup> | Lbs./ton | Concentrate     |               | Tails per cent copper | Copper recovery per cent in concentrate | Iron recovery per cent in concentrate |
|-------------------------------------|----------|-----------------|---------------|-----------------------|-----------------------------------------|---------------------------------------|
|                                     |          | Per cent copper | Per cent iron |                       |                                         |                                       |
| Ethyl R. P. in cresylic acid        | 0.033    | 14.4            | 23.8          | 0.14                  | 86.14                                   | 45.82                                 |
| Isopropyl R. P. in cresylic acid    | 0.033    | 14.1            | 24.2          | 0.15                  | 85.53                                   | 47.97                                 |
| Second butyl R. P. in cresylic acid | 0.033    | 13.9            | 24.0          | 0.145                 | 86.07                                   | 47.64                                 |
| Pentasol R. P. in cresylic acid     | 0.033    | 14.1            | 24.5          | 0.15                  | 84.84                                   | 47.71                                 |
| Ethyl R. P. in pentasol             | 0.033    | 14.6            | 25.0          | 0.13                  | 86.55                                   | 48.55                                 |
| Isopropyl R. P. in pentasol         | 0.033    | 13.7            | 24.9          | 0.13                  | 87.48                                   | 53.23                                 |
| Second butyl R. P. in pentasol      | 0.033    | 14.1            | 24.5          | 0.14                  | 86.20                                   | 50.34                                 |
| Pentasol R. P. in pentasol          | 0.033    | 14.6            | 25.0          | 0.135                 | 86.59                                   | 49.9                                  |
| Diethylcarbinol R. P. in pentasol   | 0.033    | 14.0            | 24.0          | 0.135                 | 86.63                                   | 51.74                                 |
| Xanthate                            | 0.035    | 11.5            | 27.6          | 0.13                  | 85.1                                    | 62.2                                  |

R. P. flotation reagents were prepared from an alcohol, benzoylchloride and NaCNS; only the alcohol is indicated in the tabulation. R. P.'s were used in form of 33.3% R. P. to 66.7% cresylic acid and 1-1 R. P. in pentasol and freed from the alkali halide by filtration.

<sup>1</sup> Cresylic acid fuel oil mix used as frother.

An increased copper recovery and a concentrate containing less iron shows the greater selectivity of the "R. P." flotation agents.

proportions. All of these preparations were used on a Utah sulphide copper ore as shown in the 75 subjoined tabulation.

Tabulation #5.—Copper ore from Utah

| Flotation reagents used—<br>0.02 lb./ton of ore with<br>cresylic acid as a<br>frother | Concentrate           |                     | Tails<br>ings<br>per<br>cent<br>copper | Copper<br>re-<br>covery<br>per<br>cent in<br>concen-<br>trate | Iron<br>re-<br>covery<br>per<br>cent in<br>concen-<br>trate | 5  | Flotation reagent                         | Lbs./ton | Recovery, per<br>cent concen-<br>trates |      |      | Recovery, per<br>cent tailings |     |      |
|---------------------------------------------------------------------------------------|-----------------------|---------------------|----------------------------------------|---------------------------------------------------------------|-------------------------------------------------------------|----|-------------------------------------------|----------|-----------------------------------------|------|------|--------------------------------|-----|------|
|                                                                                       | Per<br>cent<br>copper | Per<br>cent<br>iron |                                        |                                                               |                                                             |    |                                           |          | Pb                                      | Zn   | Fe   | Pb                             | Zn  | Fe   |
| (a) K. salt isopropyl R. P., 60%; pentasol xanthate, 40%.                             | 20.6                  | 14.9                | 0.10                                   | 90.5                                                          | 25.0                                                        | 10 | Pot. salt isopropyl re-<br>action product | 0.04     | 80.4                                    | 7.8  | 4.3  | —                              | —   | —    |
| (b) K. salt isopropyl R. P., 60%; pentasol xanthate, 40%.                             | 18.6                  | 12.1                | 0.12                                   | 89.2                                                          | 22.9                                                        | 10 | Do                                        | 0.15     | 10.1                                    | 85.5 | 13.2 | 9.5                            | 6.7 | 82.5 |
| (c) K. salt isopropyl R. P., 60%; pentasol xanthate, 40%.                             | 20.6                  | 13.2                | 0.12                                   | 89.5                                                          | 22.2                                                        | 15 | Pot. salt 20% butyl re-<br>action product | 0.04     | 81.2                                    | 8.0  | 4.7  | —                              | —   | —    |
| (d) K. salt isopropyl R. P., 60%; pentasol xanthate, 40%.                             | 18.4                  | 15.5                | 0.10                                   | 91.6                                                          | 30.1                                                        | 15 | Do                                        | 0.15     | 8.2                                     | 85.6 | 12.5 | 10.6                           | 5.4 | 82.8 |
| K. salt isopropyl R. P., 100%.                                                        | 22.4                  | 13.7                | 0.12                                   | 89.1                                                          | 21.2                                                        | 15 | Pot. salt pentasol re-<br>action product  | 0.04     | 82.1                                    | 8.1  | 4.6  | —                              | —   | —    |
| Pentasol xanthate, 100%.                                                              | 16.8                  | 21.1                | 0.12                                   | 89.9                                                          | 43.8                                                        | 15 | Do                                        | 0.15     | 8.7                                     | 87.7 | 13.7 | 9.2                            | 4.2 | 81.7 |
| K. salt isopropyl R. P., 80%; ethyl xanthate, 20%.                                    | 20.6                  | 13.9                | 0.12                                   | 89.3                                                          | 24.7                                                        | 20 | Ethyl xanthate                            | 0.04     | 92.1                                    | 11.6 | 8.1  | —                              | —   | —    |
| K. salt isopropyl R. P., 60%; ethyl xanthate, 40%.                                    | 19.4                  | 16.6                | 0.12                                   | 89.2                                                          | 30.7                                                        | 20 | Do                                        | 0.15     | 4.7                                     | 86.6 | 16.5 | 3.2                            | 1.8 | 75.4 |
| K. salt isopropyl R. P., 40%; ethyl xanthate, 60%.                                    | 18.4                  | 18.8                | 0.12                                   | 89.4                                                          | 37.3                                                        | 25 | Minerec A                                 | 0.034    | 91.4                                    | 11.0 | 7.4  | —                              | —   | —    |
| K. salt isopropyl R. P., 20%; ethyl xanthate, 80%.                                    | 17.2                  | 21.4                | 0.12                                   | 89.3                                                          | 43.7                                                        | 25 | Ethyl xanthate                            | 0.154    | 5.7                                     | 86.6 | 15.8 | 2.9                            | 2.4 | 76.8 |
| Ethyl xanthate, 100%.                                                                 | 15.8                  | 19.9                | 0.11                                   | 90.2                                                          | 46.4                                                        | 25 | Minerec A                                 | 0.34     | 92.5                                    | 11.8 | 8.1  | —                              | —   | —    |
| K. salt isopropyl R. P., 100%.                                                        | 23.6                  | 15.0                | 0.13                                   | 88.4                                                          | 23.3                                                        | 20 | Pot. salt pentasol re-<br>action product  | 0.154    | 4.8                                     | 87.0 | 13.4 | 2.7                            | 1.2 | 78.5 |

## LEGEND:

- (a) Wet K. salt of isopropyl R. P. mixed with commercial pentasol xanthate dried.  
 (b) Wet K. salt of isopropyl R. P. mixed with pentasol xanthate ingredients dried.  
 (c) Isopropyl reaction product mixed with pentasol, CS<sub>2</sub> and enough KOH to form double salt and dried.  
 (d) Dry K. salt of isopropyl R. P. mixed with commercial pentasol xanthate.

To show the selective action of the reagents of this invention upon sulphide lead and sulphide zinc minerals over sulphide iron mineral as compared with xanthates, a series of tests were made on a lead-zinc ore from Idaho.

The procedure followed consisted in taking off a lead concentrate by means of a small amount of collecting agent and the usual cresylic acid frother and after conditioning with copper sulphate and additional collecting agent, a zinc concentrate was taken off. This is shown in Tabulation No. 6, less iron and more lead and zinc being recovered with the "R. P." agent than with the xanthate or Minerec A, a xanthic acid formate as made under the Fischer Patent 1,684,536.

Tabulation #6.—Lead-zinc ore from Idaho

## A

| Flotation reagent                         | Lbs./ton | Assays, per cent<br>concentrates |      |     | Assays, per cent<br>tailings |      |      |
|-------------------------------------------|----------|----------------------------------|------|-----|------------------------------|------|------|
|                                           |          | Pb                               | Zn   | Fe  | Pb                           | Zn   | Fe   |
| Pot. salt isopropyl re-<br>action product | 0.04     | 57.6                             | 8.1  | 4.4 | —                            | —    | —    |
| Do                                        | 0.15     | 3.4                              | 42.6 | 6.4 | 0.45                         | 0.46 | 5.5  |
| Pot. salt 20% butyl re-<br>action product | 0.04     | 55.4                             | 8.1  | 4.6 | —                            | —    | —    |
| Do                                        | 0.15     | 2.8                              | 43.6 | 6.2 | 0.48                         | 0.36 | 5.5  |
| Pot. salt pentasol re-<br>action product  | 0.04     | 55.3                             | 8.1  | 4.4 | —                            | —    | —    |
| Do                                        | 0.15     | 2.8                              | 42.0 | 6.4 | 0.43                         | 0.29 | 5.4  |
| Ethyl xanthate                            | 0.04     | 50.2                             | 9.4  | 6.3 | —                            | —    | —    |
| Do                                        | 0.15     | 1.5                              | 40.5 | 7.4 | 0.15                         | 0.13 | 5.1  |
| Minerec A                                 | 0.034    | 52.1                             | 9.6  | 6.3 | —                            | —    | —    |
| Ethyl xanthate                            | 0.154    | 1.88                             | 44.0 | 7.8 | 0.13                         | 0.16 | 5.05 |
| Minerec A                                 | 0.34     | 51.6                             | 9.6  | 6.3 | —                            | —    | —    |
| Pot. salt pentasol re-<br>action product  | 0.154    | 1.73                             | 45.8 | 6.8 | 0.13                         | 0.08 | 5.3  |

6. The improvement in the concentration of ores by flotation which comprises subjecting a sulphide ore in the form of a pulp to a flotation operation in the presence of an effective quantity of a froth flotation agent comprising a reaction product of an aliphatic monohydric alcohol, an alkali thiocyanate and a carbocyclic acid halide.
7. The improvement in the concentration of ores by flotation which comprises subjecting a sulphide ore in the form of a pulp to a flotation operation in the presence of an effective quantity of a froth flotation agent comprising an amyl alcohol solution of a reaction product of an aliphatic monohydric alcohol, an alkali thiocyanate and a carbocyclic acid halide.
8. The improvement in the concentration of ores by flotation which comprises subjecting a

sulphide ore in the form of a pulp to a flotation operation in the presence of an effective quantity of a froth flotation agent comprising a water soluble reaction product of an aliphatic monohydric alcohol, an alkali thiocyanate, a carbocyclic acid halide and an alkali hydroxide.

9. The improvement in the concentration of ores by flotation which comprises subjecting a sulphide ore in the form of a pulp to a flotation operation in the presence of an effective quantity of a froth flotation agent comprising (1) a reaction product of an aliphatic monohydric alcohol, an alkali thiocyanate, and a carbocyclic acid halide and (2) an alkali metal xanthate of a monohydric aliphatic alcohol.

10. The improvement in the concentration of ores by flotation which comprises subjecting a

sulphide ore in the form of a pulp to a flotation operation in the presence of an effective quantity of a froth flotation agent comprising (1) a reaction product of an aliphatic monohydric alcohol, an alkali thiocyanate, and a carbocyclic acid halide and (2) an alkali metal salt of an alkyl sulphur derivative of carbonic acid.

11. The improvement in the concentration of ores by flotation which comprises subjecting a sulphide ore in the form of a pulp to a flotation operation in the presence of an effective quantity of a froth flotation agent comprising (1) a reaction product of an aliphatic monohydric alcohol, an alkali thiocyanate, and a carbocyclic acid halide and (2) an alkyl sulphur derivative of carbonic acid.

CORNELIUS H. KELLER.